

Aug. 31, 1943.

A. G. TULL

2,328,368

COLOR PHOTOGRAPHY AND CINEMATOGRAPHY

Filed March 19, 1941

FIG. 1.



FIG. 2.



Inventor  
Alan G. Tull,  
B.B. Bellings  
Attorney

## UNITED STATES PATENT OFFICE

2,328,368

COLOR PHOTOGRAPHY AND  
CINEMATOGRAPHY

Alan Gilbert Tull, Purley, England, assignor to  
Latta Syndicate Limited, London, England, a  
British company

Application March 19, 1941, Serial No. 384,180  
In Great Britain March 27, 1940

5 Claims. (Cl. 95—2)

The present invention relates to methods of producing multi-color photographic records, and more especially records made through the processing of a photographic material such as that disclosed in my co-pending application filed October 24, 1941, Serial No. 416,407, which is a division of the present application, whereby to produce either natural color positives, or master records, either negative or positive, which are not necessarily natural color records of the original subject but from which natural color prints may be made.

The invention has for its principal object, to provide a simple, relatively inexpensive and satisfactory method of producing a multi-color photographic record on a material comprising a support carrying at least three silver halide emulsion layers, of which layers the one nearest the support is diffusely dyed with a dye capable of being processed by the silver dye-bleach process to form a color image, while the other layers are substantially colorless.

Briefly stated, the process constituting the present invention, as applied to such a material, comprises its exposure, and development of the latent images to silver; its treatment to form image deposits in its layers which are suitable for chemical toning; its further treatment in a mixed toning bath to form differently-colored chemically-toned images in some of its layers; and its treatment to produce a dye image in the diffusely dyed layer by dye destruction, at any stage at which there is a silver image in said diffusely dyed layer.

Various specific modes of carrying out the invention are described more fully below, both as regards processing by reversal and by negative technique to give a negative record from which copies may be made by printing; and in order that the invention may be the better understood, reference is made to the accompanying drawing constituting a part of this specification, in which there is diagrammatically illustrated two forms of the material referred to above and which is more fully described and claimed in my said co-pending application Serial No. 416,407.

In the said drawing:

Fig. 1 represents a form of material suitable for processing either by reversal to form a natural color positive or by non-reversal procedure to form a complementarily colored negative.

Fig. 2 represents forms of material suitable for the production of a non-complementary positive or negative master record and for copying such records.

In the form shown in Fig. 1, a Celluloid support 1 is coated with an emulsion layer 2 which is blue sensitive and diffusely dyed yellow, followed by a green sensitive layer 3, and a red sensitive layer 4. A red or green absorbing filter layer 5, which is destroyed or removed during the processing of the material may be required if the layer 4 is also green sensitive.

In the form shown in Fig. 2 a transparent support 1, is coated with a red sensitive layer 6 which is colored yellow, followed by a green sensitive layer 7 and a blue sensitive layer 8. A yellow filter layer 9 is preferably interposed between the layers 7 and 8 while a red filter layer 10 may be provided between the layers 6 and 7.

In another form the layer 6 is green sensitive and diffusely colored magenta, the layer 7 is red sensitive and layer 8 blue sensitive. In this case the filter layer 10, if required, is of green color.

In the production of duplicate copies or prints from master positive or negative records produced on the material shown on Fig. 2, in which the blue sensitive layer is processed blue-green as described below while the middle layer is colored either magenta or yellow according to whether the lowermost layer is diffusely dyed yellow or magenta respectively, copying is effected on a similar type material.

In the case of a copying material the support 1 may be of translucent or opaque material such as paper, forming the final support of the colored print.

The first step in the processing of the material after exposure is to develop the latent images in the different layers to silver. This is preferably performed in an ordinary negative developer, which in the case of reversal processing contains a proportion of a silver solvent such as potassium thiocyanate. Further steps are dependent on whether a positive or negative is to be produced. In the case of the production of a positive by reversal the form of material indicated above in Fig. 1 is exposed through the support and after development further steps include the conversion of the residual halide into an intermediate in the formation of a colored image by chemical toning and the selective destruction of the dye-stuff in the bottom layer at the points occupied by the developed silver therein. In my co-pending application filed February 10, 1941, Serial No. 378,301 a process of producing such an intermediate is described wherein the conversion is performed directly in a bath containing a substance capable of forming a complex with the halide which complex is then converted into the inter-

mediate. Thiourea in acid solution is a well known reagent for the production of color images by the silver dye-bleach process and it has been found that the conversion bath given in the aforesaid application No. 378,301 may be modified by the addition of an acid such as sulphuric acid and preferably also of hydroquinone without modifying the characteristics of such bath as regards the conversion of the residual halide into a silver ferrocyanide and that such modified bath then serves also for the selective destruction of the dyestuff in the bottom layer.

As a result of the processing steps so far described there are in the top two layers reversed image deposits of silver ferrocyanide or a complex thereof and in the bottom layer a reversed yellow color image produced by the selective destruction of the dyestuff at the points occupied by the silver image therein; there may also be a deposit of silver ferrocyanide but this is unaffected by the further processing.

As described in my co-pending application filed February 10, 1941, Serial No. 378,302 such intermediate images may be treated in a mixed toning bath preferably containing a ferric salt and a uranium salt whereby a deposit of Prussian blue is formed in a surface layer and a deposit of uranium ferrocyanide below forming a red image. It has been discovered that by suitable control in the proportions of the constituents of the mixed bath, particularly in the amount of potassium bromide, as explained in the aforesaid application No. 378,302, the effect of the mixed toning bath may be confined to the top two layers of the material so that any silver ferrocyanide which may be in the bottom layer is unaffected. The final step is to remove silver and silver salts in the several layers in Farmer's reducer or in the modified form of this reagent mentioned in said last mentioned application.

Inasmuch as the uranium ferrocyanide image is not fully satisfactory as the magenta image of a three color record, preferably the material is treated in a solution of a soluble zinc salt which converts the uranium salt into zinc ferrocyanide which is dye-toned with a suitable magenta dye as described in my co-pending application filed April 3, 1941, Serial No. 386,744.

In the processing to form a negative master record on any of the forms of material referred to above after development of the latent images, the silver images are converted into silver ferrocyanide or other suitable intermediate in view of the further processing steps, without fixing the layers. To this end the following bleach may be used:

|                            | Cubic centimeters |
|----------------------------|-------------------|
| Potassium ferricyanide 10% | 12                |
| Ammonia (.880)             | 1.2               |
| Water to                   | 60                |

Further steps include the treatment of the material in a mixed toning bath, particularly one containing a ferric salt and a uranium salt, and so controlled that only the two outer layers are affected, and treatment in a bath which produces a colored negative in the pre-dyed bottom layer. It will be observed that the condition laid down in application No. 378,302, that the intermediate image in the two outer layers is surrounded by a complementary deposit, is still maintained. As an alternative to preliminarily bleaching the silver and then treating in a toning bath, a combined bath could be used, that is one containing beside the toning reagents a

5 proportion of potassium ferricyanide. The production of the negative image in the pre-dyed layer may be performed at any stage in the processing, where the developed latent image remains as silver in that layer, in a bath which destroys the dye at the points not occupied by the said silver. Such a bath is, for instance, the following:

|                      |       |     |
|----------------------|-------|-----|
| Calcium hypochlorite | gms-- | 2   |
| Glacial acetic acid  | ccs-- | 2   |
| Water to             | ccs-- | 200 |

10 The uranium ferrocyanide image in the middle layer may, if desired, be replaced by a dye-toned image, as referred to above, said dye-toned image being either magenta or yellow according to the type of material used.

15 If a photographic material is used for the production of a negative comprising a support carrying in succession a blue-sensitive, yellow dyed emulsion, a green sensitive emulsion, colored magenta during processing, and a red sensitive emulsion colored blue-green during processing, exposure being effected through the support, the record obtained embodies part images which are 20 colored complementarily to the color aspect of which the image is a record in each case and such material is obviously capable of being copied onto a similar copy material but in such case the copy material is exposed through the support although the master record may face either way during the printing operation. Such printing 25 may be performed with white light or successively with different colored lights the spectral properties of which are such that printing is performed correctly in the several layers of the copy material.

30 If, as shown in Fig. 2, the negative material includes a support carrying in succession a red sensitive layer colored yellow, a green sensitive layer and a blue sensitive layer, exposure being 35 performed from the front, a record is obtained in which the blue of the original object is rendered as Prussian blue, i. e., blue-green, the green is recorded as magenta and the red as yellow. Such a master may be printed onto a similar copy material from the front, i. e., emulsion side thereof, either with white light or with colored lights in succession.

40 Forms of the material described herein intended for use as copy material and for use in the production of a positive by reversal may include a stripping layer between the emulsion layers and the base to enable the layers to be transferred to a new support, as described in my co-pending application Serial No. 384,182, filed March 19, 1941. Alternatively the layers could be coated on an opaque or translucent support such as paper or a layer could be interposed between the support and the emulsion layers which 45 interposed layer is opaque white. If exposure has to be made through the support or printing effected in the same manner, such support must be transparent and a layer may be interposed between the emulsion layers and the support which is initially transparent and capable of being converted into an opaque white layer during processing as described in my co-pending application Serial No. 384,181, filed March 19, 1941.

50 It is to be understood that the present invention also includes the copying of a positive natural color record produced by reversal onto a similar material and the processing of the copied record by reversal to form duplicated copies. 55 Further the invention is not restricted to the

processing of a multicoated material as three different strata of a single emulsion coat may be sensitized differently at different depths and processed as described herein.

I claim:

1. A method of producing a multi-color photographic record on a material including a support and several silver halide emulsion layers coated thereon of which the layer nearest the support is diffusely dyed with a dye capable of being discharged selectively to form a color image and the other layers are substantially colorless, comprising exposing such material, developing the latent images therein to silver, producing silver ferrocyanide images in said layer, treating the material in a toning bath containing a ferric salt and a uranium salt to form a Prussian blue image in the uppermost layer and a uranium ferrocyanide image in the following layer and, at any stage where the developed silver image in the layer nearest the support remains as silver, producing a color image in said layer by the selective destruction of the dyestuff therein.

2. A method of producing a multi-color photographic record on a material including a support and several silver halide emulsion layers coated thereon of which the layer nearest the support is diffusely dyed with a dye capable of being discharged selectively to form a color image and the other layers are substantially colorless, comprising exposing such material, developing the latent images therein to silver, producing silver ferrocyanide images in said layers, treating the material in a toning bath containing a ferric salt and a uranium salt to form a Prussian blue image in the uppermost layer and a uranium ferrocyanide image in the following layer, replacing said latter by a zinc ferrocyanide image, dye toning the latter image with a dye which mordants to the said image and, at any stage where the developed image in the layer nearest the support remains as silver, producing a color image in said layer by the selective destruction of the dyestuff therein.

3. A method of producing a natural color positive photographic picture on a material including a transparent support, a blue sensitive yellow dyed layer of photographic silver halide emulsion coated on said support and green and red sensitive emulsion layers coated in turn on said blue sensitive layer, comprising exposing such material through the support, developing the latent images formed in said layers, converting the residual halide in such layers into a silver ferro-

cyanide, toning the latter in a mixed toning bath containing a ferric salt and a uranium salt to form a Prussian blue image in the surface layer and a uranium ferrocyanide image in the following layer and, at any stage where the developed silver image in the layer nearest the support remains as silver, producing a color image in the yellow dyed layer by the selective destruction of the dyestuff therein.

4. A method of producing a master multi-color photographic record from which natural color prints can be produced, employing as exposure material a multi-layer element having a support, a layer thereon which is diffusely dyed with a dyestuff which is capable of being discharged selectively to form a color image and two further layers sensitive to different colors, the outermost layer being blue sensitive, comprising exposing such material from the emulsion side, developing the latent images formed in the layers, bleaching the developed images to silver ferrocyanide, toning the latter in a mixed toning bath containing a ferric salt and a uranium salt to form a Prussian blue image in the surface layer and a uranium ferrocyanide image in the following layer, and, at any stage where the developed image in the layer nearest the support consists of silver, producing a color image in said layer by the selective destruction of the dyestuff therein at the points unoccupied by the developed silver image.

5. In the production of a multi-color photographic copy from a multi-color photographic master record, employing as copy material a multi-layer element having a support, a blue-sensitive emulsion layer thereon which is diffusely dyed with a dyestuff which is capable of being discharged selectively to form a color image, and two further substantially colorless emulsion layers sensitive to different colors, the method which comprises printing such copy material from the master record through the support of the copy material; developing the latent images formed in the layers; producing silver ferrocyanide images in said layers; treating the material in a toning bath containing a ferric salt and a uranium salt to form a Prussian blue image in the uppermost layer and a uranium ferrocyanide image in the following layer; and, at any stage where the developed silver image in the layer nearest the support remains as silver, producing a color image in said layer by the selective destruction of the dyestuff therein.

ALAN GILBERT TULL.